

## UNITED STATES PATENT OFFICE

2,423,020

PROCESS FOR TREATMENT OF LUMBER  
AND OTHER FOREST PRODUCTSJoye C. Haun, San Francisco, Calif., assignor to  
Electric Steel Foundry, Portland, Oreg., a cor-  
poration of OregonNo Drawing. Application April 7, 1944,  
Serial No. 530,062

13 Claims. (Cl. 260—110)

2

The present invention relates to processes for treatment of lumber and other forest products, and is particularly concerned with the solvent treatment of wood for the purpose of obtaining uniform moisture content in the wood and in order to remove the pitches and resins, and other soluble constituents from the wood.

In the sulphite pulp process it is important that the moisture content of the wood to be cooked be uniform. It is also important that the pitch and resin content of the wood be as low as possible.

Wood which is too dry is very difficult to cook without charring and discoloration. Pitch causes foaming in the digester and consumes acid. The removal of the pitches and resins and the adjustment of the moisture content to a predetermined uniform percentage will give a superior cellulose pulp to that which can be obtained by the use of untreated wood. In addition to the improvement of the wood product for pulp, the resins and pitches, and other by-products removed from the wood may have a value which almost entirely offsets the cost of the treatment of the wood.

One of the objects of the invention is the provision of an improved method of treatment of wood by means of which the moisture content of the wood may be brought to a substantially uniform amount in order to render the wood in the best possible condition for use in the sulphite pulp process.

Another object of the invention is to render pitchy wood of variable moisture content suitable for cellulose fiber manufacture.

Another object of the invention is to render logging slash more suitable for sulphite treatment by adjusting the moisture content and distributing the moisture uniformly to each individual piece of wood so that the moisture content will be uniform.

Another object of the invention is the provision of an improved process for adjusting the moisture content in chips of any sort of wood and for removing the pitches and resins so as to condition the chips to be more easily and completely digested by sulphite liquor.

Another object of the invention is the provision of an improved method of treatment of wood by means of a three-component solvent which is adapted to dissolve the pitch and resin in the wood more quickly and more readily and in greater amounts than the processes of the prior art and which permits the quick and easy recovery of the pitches and resins from the solution.

Another object of the invention is the provision of an improved and simple, economical method of recovery of the soluble constituents of wood in a relatively pure form and separated from each other.

Other objects and advantages of the invention will be apparent from the following description; but, as the present process may be carried out by the use of many different standard types of apparatus of the prior art, no drawing is required to illustrate the invention.

The solvent employed in my method of treating wood is preferably a solvent having three components, one of which is an organic, aliphatic solvent that is miscible with water, such as, for example, acetone. Other solvents that may be used are alcohol, methanol, and the like; but acetone is preferred, and the invention will be described with respect to the use of acetone.

15 The other two components of the solvent are preferably carbon tetrachloride and water, and in general the carbon tetrachloride may be replaced by any other solvent which will form a solution with acetone and which solvent per se is immiscible in the acetone-water solution, such as, for example, trichlorethylene, trichlorethane, or chloroform.

20 Considering cost and all other factors, the carbon tetrachloride is the other constituent solvent which I prefer to use with acetone and water in carrying out my process.

25 The proportions of the various components in the solvent solution may be varied. For example, the solution may include fifty percent of acetone and fifty percent of water, and added to this mixture there may be carbon tetrachloride in the amount of ten percent of the volume of the acetone. More than fifty percent of water content is preferably not employed, as the rapidity with

30 which pitch goes into solution is somewhat retarded by increased water content, and also in order to avoid the necessity for later distillation of the water-acetone solution; and in general only sufficient water is preferably employed to form an acetone-carbon tetrachloride solution and a water-acetone solution, the two being immiscible.

35 As one of the functions of the present treatment is to adjust the moisture content of the product, the amount of water used in the solution depends upon the moisture content which is desired in the finished product. In all cases the strength of the acetone-water solution, before its application to the wet lumber, should be predetermined from the moisture content which is 40 desired in the finished product. The moisture

content of the finished product would be substantially the same as the moisture content of the solution as it emerges from final treatment with the lumber. This naturally may differ from the initial moisture content of the solution if a considerable amount of water is given off by the lumber or a considerable amount of water is taken on by the lumber. Therefore, the wet or dry condition of the lumber to be treated should also be taken into consideration so that when the treatment has been finished the moisture content will be that which is desired.

Naturally, if a twenty-five percent moisture content is desired in the finished wood instead of a forty-five percent moisture content, the initial amount of water in the original acetone-carbon tetrachloride water solution would be less than if a forty-five percent moisture content were desired in the finished wood. The actual water content in the solution may be slightly greater or less than the desired moisture content of the finished wood, depending on the relative wetness or dryness of the lumber being treated.

As to the range of percentages for the constituents of the solution, good results can be obtained when a start is made on wet lumber by using a solution carrying from ninety-five percent to fifty percent acetone relative to the water by volume with from five percent to twenty percent of carbon tetrachloride or other similar chemical substance relative to the volume of the acetone. These results are due to the fact that the acetone immediately withdraws water from the wet wood, which causes the carbon tetrachloride to separate out of the solution, and naturally the pitch is extracted out of the solution with the carbon tetrachloride.

To obtain the most rapid results, a solution of approximately eighty percent acetone relative to a water content by volume would be the most effective. However, the effectiveness of the acetone solution is retarded very slightly down to a fifty percent water content when in the presence of carbon tetrachloride.

The effectiveness of the removal of pitch by the solution increases as the amount of water in the solution is diminished, and decreases as the amount of water in the solution is increased; but the solution is still very effective when as much as fifty percent water by volume relative to the acetone content exists in the solution. The water content, however, is preferably determined by the water content desired in the finished product; but when the amount of water content in the finished product is of no consideration, then the rapidity of pitch removal may be increased by diminishing the amount of water so that the proportion of acetone relative to water by volume may be as high as eighty percent acetone, or even higher.

A composite solvent of this nature forms two separate solutions, water-acetone solution, and acetone-carbon tetrachloride solution. These two solutions do not mix, and are easily separated, although there are very minor quantities of carbon tetrachloride in the water-acetone solution and very minor quantities of water content in the acetone-carbon tetrachloride solution.

The solubility of pitch in acetone is a function of the purity of the acetone; and when water is present, the limit of solubility of the pitch decreases with increasing water content. The solubility of pitch in acetone-carbon tetrachloride is greater than in water-acetone solution, as the water content of the acetone-carbon tetrachloride

solution is very low under all conditions, and both acetone and carbon tetrachloride are extremely good solvents for pitch.

Carbon tetrachloride alone is not a good solvent for pitch from wet wood, as it will not penetrate into the wood, due to the relative insolubility of carbon tetrachloride in water and the low solubility of water in carbon tetrachloride. However, in a mixture consisting of acetone, carbon tetrachloride, and water, the water-acetone solution penetrates the chips and rapidly dissolves the pitch to its soluble limit. The dissolved pitch is then rapidly transferred from the water-acetone solution to the acetone-carbon tetrachloride solution.

This continually reduces the amount of dissolved pitch in the water-acetone solution so that this solution may continue to penetrate the chips and to dissolve the pitch from the wood.

Under these conditions, therefore, the water-acetone mixture can never become saturated as long as the acetone-carbon tetrachloride solution can continue to take up the pitch from the water-acetone solution and the maximum dissolving efficiency of the water-acetone solution is maintained.

I have found that the pitch content of the acetone-carbon tetrachloride solution can be built up to a very high percentage without in any way retarding the dissolving tendency of the water-acetone component of the mixture. This would not be the case if water and acetone were used alone without carbon tetrachloride.

In the practice of the method, pitchy stumps or butt cuts, or other forms of wood may first be prepared in a form suitable for washing with the solution.

This preparation consists of either chipping or hogging the wood. The ultimate fineness is dependent to a great extent on the nature of the wood and the amount of pitch and/or resins the wood contains.

After reducing the wood to the required size of particles, it is charged into an extractor and humidifying chamber, which consists of a tank that can be sealed from the atmosphere. The tank is then preferably closed, and the tank preferably purged of oxygen by either an inert gas or steam, the air being removed in order to eliminate the danger of forming an explosive mixture with acetone vapors in the tank.

The tank may then be filled with the pre-adjusted solution of acetone-water and carbon tetrachloride. The relative proportions of acetone and water should be such that there will be no tendency for moisture to be withdrawn from the wood at more than a given desired percentage.

Wood below this moisture content will withdraw water from the water-acetone solution, while wood having more than the desired content of water will give up water to the water-acetone solution. This transfer of water from one wood particle to another will be accelerated by the removal of pitchy and resinous material from the wood. The chips may be soaked for a predetermined time in the three-component solution, or the solution may be continuously passed over the comminuted wood or wood chips and withdrawn from the bottom of the chamber in which the chips are being treated.

This is continued, the liquid being withdrawn and replaced by fresh liquid until the material issuing from the bottom of the tank is substantially free from dissolved pitches.

The specific gravity of acetone-tetrachloride solution is much greater than that of the water-acetone solution, so that the acetone-carbon tetrachloride solution readily separates from the water-acetone solution by gravity, and can be withdrawn from a separatory funnel with the pitch which it contains.

The water soluble constituents removed from the wood in the extraction chamber will remain with the water-acetone solution; and, if desired, these can be recovered in a residue by distillation of the water-acetone solution.

The pitches can be recovered from the acetone-carbon tetrachloride solution by distillation of this solution for the recovery of the pitch, and the distilled solvents may be returned to the chips. If it is not desired to recover the water soluble constituents of the water-acetone solution which passes out of the top of the separatory funnel, this solution may be returned directly to the chips.

Thus, the recovery of the dissolved pitch is greatly facilitated by the fact that the pitch is contained in the acetone-carbon tetrachloride solution having the greater specific gravity.

While I prefer to add the carbon tetrachloride component of the solution directly to the extraction chamber, in some modes of practice of the invention the wood may be treated first with the acetone-water solution. After this solution is withdrawn from the chamber for the removal of distilled pitch, sufficient carbon tetrachloride may be added to the withdrawn solution to separate the pitch from the solution by reason of the selective solvent action of this chlorinated solvent.

The continuous transfer of pitch from the water-acetone solution, to the acetone-carbon tetrachloride solution greatly increases the dissolving action of the acetone-water solution; and therefore it is preferred to apply the three-component solvent directly to the wood that is being treated.

In general, the water-acetone solution withdrawn from the chips would not need to be distilled, unless the water content exceeds fifty per cent. The solvent remaining in the chips may be driven off by the use of live steam with a simple reflux condenser in which only part of the water would be condensed, as I do not prefer a solution of more than eighty per cent acetone.

The acetone-carbon tetrachloride vapors would be condensed in the extraction chamber, and this would tend to heat the solutions in the chamber, making the pitches more soluble in the solvents.

The temperatures at which the processes may be carried out may be varied considerably, the application of extraneous heat increasing the tendency toward solubility of the pitches, but also increasing the tendency toward production of acetone vapors and carbon tetrachloride vapors. I prefer to carry out the process without the application of extraneous heat, except that it may be introduced by the use of live steam in driving the air out of the chamber or in removing the solvent from the treated chips.

The present process is thus adapted to provide a simple economical method of recovery of the acetone-carbon tetrachloride soluble constituents of the wood, as well as the water-acetone-soluble constituents in a relatively pure form and separated from each other.

The three-component mixture will dissolve the pitch from wet wood much more readily than commercial acetone or a solution of acetone and

water. The pitch can be concentrated in a relatively small volume by the use of the carbon tetrachloride in limited quantities, as substantially all the pitch is contained in the acetone-carbon tetrachloride solution.

The use of a non-inflammable solvent, such as carbon tetrachloride and chlorinated solvents, tends to reduce the fire hazard in the extraction apparatus, but my invention includes the use of other organic solvents mentioned above, which may be inflammable and which accomplish the same results.

The moisture content in the wood that has been treated is substantially uniform throughout the various particles of the wood; and the pitch having been removed, the treated wood is in the best condition to be used to produce a superior cellulose pulp.

As the constituents of the solvent mixture may be used over and over again, the present process is economical in the use of materials.

While I have illustrated a preferred embodiment of my invention, many modifications may be made without departing from the spirit of the invention, and I do not wish to be limited to the precise details of the process set forth, but desire to avail myself of all changes within the scope of the appended claims.

Having thus described my invention, what I claim as new and desire to secure by Letters Patent of the United States, is:

1. The method of treatment of wood for the removal of the pitch which comprises subjecting the wood to the dissolving action of water and acetone to dissolve the pitch, and segregating the pitch from the water-acetone solution by the action of carbon tetrachloride in an amount of 5% to 20% by volume of the acetone, which combines with part of the acetone to form an acetone-carbon tetrachloride solution to which the pitch is transferred from the water-acetone solution.

2. The method of treatment of wood for the removal of the pitch which comprises subjecting the wood to the dissolving action of water and acetone to dissolve the pitch, and segregating the pitch from the water-acetone solution by the action of carbon tetrachloride in an amount of 5% to 20% by volume of the acetone, which combines with part of the acetone to form an acetone-carbon tetrachloride solution to which the pitch is transferred from the water-acetone solution, and distilling the acetone-carbon tetrachloride solution to separate the pitch as a residue and to return the acetone-carbon tetrachloride liquid for further use.

3. The method of removing water-soluble constituents and pitch from wood, which comprises subjecting the wood to the action of a three-component solution containing water, acetone, and carbon tetrachloride in such manner that a water-acetone solution is formed containing the water-soluble constituents and an acetone-carbon tetrachloride solution is formed containing the pitch constituents, the pitch being dissolved out of the wood by the water-acetone solution and transferred to the acetone-tetrachloride solution.

4. The method of removing water-soluble constituents and pitch from wood, which comprises subjecting the wood to the action of a three-component solution containing water, acetone, and carbon tetrachloride in such manner that a water-acetone solution is formed containing the water-soluble constituents and an acetone-carbon

tetrachloride solution is formed containing the pitch constituents, the pitch being dissolved out of the wood by the water-acetone solution and transferred to the acetone-tetrachloride solution, and separating the latter solution from the effluent by virtue of the difference in specific gravity.

5. The method of removing water-soluble constituents and pitch from wood, which comprises subjecting the wood to the action of a three-component solution containing water, acetone, and carbon tetrachloride in such manner that a water-acetone solution is formed containing the water-soluble constituents and an acetone-carbon tetrachloride solution is formed containing the pitch constituents, the pitch being dissolved out of the wood by the water-acetone solution and transferred to the acetone-tetrachloride solution, and separating the latter solution from the effluent by virtue of the difference in specific gravity, and distilling the water-acetone effluent to remove the water-soluble constituents therefrom.

6. The method of removing water-soluble constituents and pitch from wood, which comprises subjecting the wood to the action of a three-component solution containing water, acetone, and carbon tetrachloride in such manner that a water-acetone solution is formed containing the water-soluble constituents and an acetone-carbon tetrachloride solution is formed containing the pitch constituents, the pitch being dissolved out of the wood by the water-acetone solution and transferred to the acetone-tetrachloride solution, and separating the latter solution from the effluent by virtue of the difference in specific gravity, and distilling the acetone-carbon tetrachloride effluent to separate the pitch from the distillate.

7. The method of extracting pitch from wood in which the wood is treated with a water solution of an aliphatic, water-soluble solvent for pitch and simultaneously removing the pitch from the first mentioned solvent by a second pitch solvent soluble in the organic aliphatic solvent but insoluble in water, thereby constantly regenerating the primary pitch solvent and accelerating the removal of the pitch from the wood.

8. The method of treating wood, which comprises subjecting the wood to a water solution containing a solvent for pitch and other soluble constituents of wood, and simultaneously segregating the pitch from the solvent solution by means of a chlorinated organic aliphatic solvent for pitch which is immiscible with water and miscible with the first-mentioned solvent.

9. The process of treating wood which comprises the steps of determining the moisture content of the wood before treatment, subjecting the wood to a water solution containing a water soluble solvent for pitch and other soluble constituents of the wood and the water content of which solution is predetermined in relation to the determined moisture content of the wood to produce a desired moisture content in the wood after treatment, and simultaneously separating said pitch and other soluble constituents from the solvent solution by the agitation therewith of a chlorinated organic aliphatic solvent for pitch which is immiscible with water and miscible in the said water soluble solvent.

10. The process of treating wood which comprises the steps of determining the moisture content of the wood before treatment, subjecting the wood to a water solution of acetone having a percentage of water determined in relation to that of the wood to provide the desired moisture content in the treated wood, and simultaneously admixing with the acetone solution a chlorinated organic aliphatic solvent for pitch which is miscible with the acetone and immiscible in water, the admixed amount of said chlorinated organic aliphatic solvent being between 5% and 20% by volume of the acetone.

11. The method of treatment of wood for the removal of the pitch which comprises subjecting the wood to the dissolving action of water and acetone to dissolve the pitch, and simultaneously segregating the pitch from the water-acetone solution by the action of carbon tetrachloride in the amount of 5% to 20% by volume of the acetone to regenerate the acetone during its pitch dissolving action upon the wood, allowing the carbon tetrachloride pitch solution to separate by gravity from the water-acetone-carbon tetrachloride mixture, draining off the separated carbon tetrachloride-pitch solution and distilling the carbon tetrachloride-pitch solution to separate the pitch as a residue and reclaim the carbon tetrachloride.

12. The method of treating wood, which comprises the steps of subjecting the wood to a water solution containing a primary water soluble solvent for pitch and other soluble constituents of wood, and simultaneously segregating the pitch from the primary solvent solution during its action upon the wood by means of the agitation therewith of a chlorinated organic aliphatic solvent for pitch which is immiscible with water and miscible with said primary solvent.

13. The method of treating a pitch extraction solution containing water, acetone and pitch while said solution is in direct contact with wood from which pitch has been extracted and which comprises subjecting the said solution to the action of a chlorinated aliphatic hydrocarbon solvent which is miscible with said acetone and immiscible in water for removing the pitch from the pitch extraction solution, thereby regenerating the said extracting solution for pitch extraction and accelerating further pitch-removing action of the extracting solution.

JOYE C. HAUN.

#### REFERENCES CITED

The following references are of record in the file of this patent:

#### UNITED STATES PATENTS

| Number     | Name          | Date          |
|------------|---------------|---------------|
| 1,389,575  | Brick _____   | Sept. 6, 1921 |
| Re. 19,749 | Bent _____    | Nov. 12, 1935 |
| 1,523,578  | Bredlik _____ | Jan. 20, 1925 |

#### OTHER REFERENCES

International Critical Tables, 1st edition, volume III, pages 418, 419, 422 and 425, pub. 1928 by McGraw-Hill Book Co. of N. Y.

Fitzgerald, "The Paper Mill," Nov. 7, 1936, pp. 16-18.

The Merck Index, fifth edition, page 4.